

## UNITED STATES PATENT OFFICE

2,584,400

PROCESS FOR ANODIC OXIDATION OF  
ALUMINUM AND ITS ALLOYS

Carlo Sonnino, Milan, Italy

No Drawing. Application May 29, 1947, Serial No.  
751,453. In Switzerland October 20, 1944Section 1, Public Law 690, August 8, 1946.  
Patent expires October 20, 1964

4 Claims. (Cl. 204—58)

1

It is known that the purpose of anodic oxidation of aluminium is to obtain very hard oxide layers which will be resistant to chemical agents.

For the anodic oxidation of aluminium and its alloys, it is known to employ baths composed of water and sulphuric acid, to which other materials may be added.

According to my invention, I have found that I can obtain very hard layers in relatively short time, if beryllium sulphate and/or beryllium salts are added to an electrolyte composed of water and sulphuric acid. The surprising feature is that layers obtained according to the invention can be colored, notwithstanding their extraordinary hardness.

The layer is colourless and transparent, vitreous and very hard, and in spite of that it can be colored by dipping or by any suitable system, either by the direct application of colors or by chemical reaction.

The time of oxidation may be from 20 minutes to an hour and the thickness of the layer obtained is 0.06 mm. The hardness is extraordinary and scleroscope hardnesses for different alloys, expressed in grams of load required for penetration of diamond tip through the whole depth of oxyde layer, are:

| Layer according to the invention | Maximum of other methods |
|----------------------------------|--------------------------|
| g.                               | g.                       |
| 225                              | 210                      |
| 236                              | 186                      |
| 194                              | 150                      |
| 145                              | 100                      |
| 110                              | 85                       |

Polyvalent alcohols can be advantageously added to the electrolytes containing beryllium sulphate or other beryllium salts according to the invention.

Two different types of layers may be obtained by varying the percentage of sulphuric acid and beryllium sulphate in the bath, namely:

1. A very hard and scarcely flexible layer suitable to prevent undesirable locking of connections, bolts or threaded elements of aluminium or its alloys to be screwed or forced in other threaded pieces of aluminium or its alloys, said layer being considerably porous so that it is possible to color, by absorption from coloring solutions, pieces intended to undergo frictional wear.

2. A less hard but very porous and flexible layer, such as will allow press-molding of oxidized articles or the formation of a colored or white

2

pigment in said layer so as to give a lacquer appearance to the objects, maintaining, however, the features of the anodic film.

Hereinafter I will describe two examples for carrying out the method according to the invention corresponding to said two types of layer:

## Example 1 (1st type layer)

10 1 kg. of beryllium sulphate is added, after cooling, to a bath composed of 15 kg. of sulphuric acid at 66° Bé. and 85.1 of distilled water.

The optimum operating range with this bath is from 13° to 21° C., with 9-15 volts (preferably 12.5 volts) and about 0.8 ampere/dm.<sup>2</sup>, aluminum 15 semi-hard plate, rolled Duralumin.

## Example 2 (2nd type layer)

15 1.5-2.5 kg. of beryllium sulphate are added, after cooling, to a bath composed of 30 kg. of sulphuric acid at 66° Bé. and 70 l. of distilled water.

20 The operating range is of 12 volts and the current density of 0.8 ampere/dm.<sup>2</sup> for rolled or drawn aluminium or aluminium alloys, or of 0.5 ampere/dm.<sup>2</sup> for cast aluminium alloys, the temperature being between 18° and 23° C., according 25 to whether color or pigment is to be absorbed.

20 Tested hardness values are somewhat smaller than in the first example and almost the same for different alloys, but still greater than those obtained by other methods: the value for aluminium, for instance, is 100 g. compared with 80 g. obtained by other methods.

Having now particularly described and ascertained the nature of my said invention and in 35 what manner the same is to be performed, I declare that what I claim is:

1. In a process for the production of transparent and hard coatings on aluminium and its alloys the step which comprises making said metal the anode in an electrolytic bath consisting 40 essentially of about 84 parts by weight of water, 15 parts of sulphuric acid and 1 part of beryllium sulphate.

2. Process as claimed in claim 1 in which said 45 bath is maintained at a temperature of 13° to 21° C. and in which the electric current passed through the bath has an intensity of about 0.8 ampere per sq. dm.

3. In a process for the production of transparent and hard coatings on aluminium and its 50 alloys the step which comprises making said metal the anode in an electrolytic bath consisting essentially of about 68 parts by weight of water, 30 parts of sulphuric acid and 1.5-2.5 parts of beryllium sulphate.

4. Process as claimed in claim 1 in which said bath is maintained at a temperature from 18° to 23° C., and in which the electric current passed through the bath has a potential of 12 volts and an intensity of 0.5-0.8 ampere per sq. dm.

CARLO SONNINO.

REFERENCES CITED

The following references are of record in the file of this patent:

UNITED STATES PATENTS

| Number    | Name     | Date          |
|-----------|----------|---------------|
| 2,018,388 | Tosterud | Oct. 22, 1935 |
| 2,022,798 | Bengston | Dec. 3, 1935  |
| 2,260,278 | Schenk   | Oct. 21, 1941 |
| 2,320,999 | Beebe    | June 8, 1943  |

FOREIGN PATENTS

| Number     | Country | Date          |
|------------|---------|---------------|
| 10 705,522 | Germany | Apr. 30, 1941 |